



US010215128B2

(12) **United States Patent**  
Smith et al.

(10) **Patent No.:** US 10,215,128 B2  
(45) **Date of Patent:** Feb. 26, 2019

(54) **ROUGH CAST CYLINDER LINER**

(71) Applicant: **MAHLE International GmbH**,  
Stuttgart (DE)

(72) Inventors: **Thomas Smith**, Muskegon, MI (US);  
**Steffen Rudolph**, Weissach (DE); **Jesús Antonio Magallanes Castañeda**, Coahuila (MX)

(73) Assignee: **MAHLE International GmbH**,  
Stuttgart (DE)

(\*) Notice: Subject to any disclaimer, the term of this patent is extended or adjusted under 35 U.S.C. 154(b) by 107 days.

(21) Appl. No.: **15/414,846**

(22) Filed: **Jan. 25, 2017**

(65) **Prior Publication Data**

US 2017/0314501 A1 Nov. 2, 2017

**Related U.S. Application Data**

(60) Provisional application No. 62/328,097, filed on Apr. 27, 2016.

(51) **Int. Cl.**

**F02F 1/00** (2006.01)  
**F02F 1/16** (2006.01)  
**F02F 1/14** (2006.01)  
**F02F 1/10** (2006.01)

(52) **U.S. Cl.**

CPC ..... **F02F 1/004** (2013.01); **F02F 1/102** (2013.01); **F02F 1/14** (2013.01); **F02F 1/163** (2013.01); **F02F 2200/06** (2013.01)

(58) **Field of Classification Search**

CPC ..... F02F 1/004; F02F 2200/06; F02F 1/14;  
F02F 1/163

USPC ..... 123/193.2, 271, 668, 669  
See application file for complete search history.

(56)

**References Cited**

**U.S. PATENT DOCUMENTS**

|              |         |               |
|--------------|---------|---------------|
| 5,855,700 A  | 1/1999  | Guerard       |
| 6,468,673 B2 | 10/2002 | Saito         |
| 6,699,314 B2 | 3/2004  | Takeo et al.  |
| 7,171,935 B2 | 2/2007  | Komai et al.  |
| 7,226,667 B2 | 6/2007  | Kodama et al. |

(Continued)

**FOREIGN PATENT DOCUMENTS**

|    |             |        |
|----|-------------|--------|
| CN | 104588572 A | 5/2015 |
| CN | 104595050 A | 5/2015 |

(Continued)

**OTHER PUBLICATIONS**

German Search Report in DE 10 2017 206 858.2 dated Feb. 27, 2018 with English translation of relevant parts.

*Primary Examiner* — Syed O Hasan

(74) *Attorney, Agent, or Firm* — Collard & Roe, P.C.

(57) **ABSTRACT**

A cylinder liner for internal combustion engines has an outer roughened surface that has particularly good adherence properties. The surface is covered with protrusions or spines of varying shapes and sizes, which are created by spraying the mold with a coating and then casting the cylinder liner in the mold. The spines are generally conical or needle-shaped, with the bases being larger than the tips. The spines have an aggregate cross-sectional surface area measured at 0.2 mm from a ground cylindrical surface that is between 50-90% of the total ground cylindrical surface area, and an aggregate cross-sectional surface area measured at 0.4 mm from the ground cylindrical surface that is between 20-45% of the total ground cylindrical surface area.

**10 Claims, 13 Drawing Sheets**



(56)

**References Cited**

U.S. PATENT DOCUMENTS

|              |      |         |                                      |
|--------------|------|---------|--------------------------------------|
| 7,383,805    | B2   | 6/2008  | Michioka et al.                      |
| 7,533,647    | B2   | 5/2009  | Miyamoto et al.                      |
| 7,665,440    | B2   | 2/2010  | Holtan et al.                        |
| 7,806,098    | B2 * | 10/2010 | Bing ..... B22D 19/0009<br>123/193.2 |
| 8,402,881    | B2   | 3/2013  | Sato et al.                          |
| 9,500,282    | B2   | 11/2016 | He et al.                            |
| 2003/0056645 | A1 * | 3/2003  | Land ..... F02F 1/004<br>123/193.2   |
| 2007/0012177 | A1   | 1/2007  | Miyamoto et al.                      |
| 2012/0304852 | A1   | 12/2012 | Yamagata et al.                      |
| 2015/0122118 | A1 * | 5/2015  | He ..... C23C 4/04<br>92/171.1       |

FOREIGN PATENT DOCUMENTS

|    |                 |    |        |
|----|-----------------|----|--------|
| CN | 204386752       | U  | 6/2015 |
| DE | 10 2004 062 527 | A1 | 7/2005 |
| DE | 10 2009 043 566 | A1 | 4/2011 |
| DE | 20 2013 100 551 | U1 | 4/2013 |

\* cited by examiner



FIG. 1

FIG. 2



FIG. 3



FIG. 4



FIG. 5

FIG. 6



FIG. 7



FIG. 8



FIG. 9



FIG. 11



FIG. 12



FIG. 13

FIG. 14



FIG. 15



FIG. 16



FIG. 17

FIG. 18



FIG. 19



FIG. 20



FIG. 21





FIG. 23

## 1

## ROUGH CAST CYLINDER LINER

## CROSS-REFERENCE TO RELATED APPLICATIONS

This application claims priority under 35 USC 119(e) of U.S. Provisional Application Ser. No. 62/328,097, filed on Apr. 27, 2016, the disclosure of which is herein incorporated by reference.

## BACKGROUND OF THE INVENTION

## 1. Field of the Invention

The present invention relates to a cylinder liner for internal combustion engines. In particular, the invention relates to a cylinder liner that has a rough exterior surface that is formed during the casting process, the surface having spines of different shape and structure to facilitate adherence of the liner to the engine block.

## 2. The Prior Art

In combustion engines having an engine block made of a cast iron alloy or an aluminum alloy, cylinder liners are usually inserted into the cylinder bores of the engine block. The liners consist of cylindrical pipe sections and their inner surfaces define the combustion space of the combustion chamber of the engine. The outer surfaces are often treated to give the outer surface a roughened texture. This rough texture ensures adhesion of the cylinder liner to the engine block when the liner is cast into the engine block.

Some cylinder liners, such as the one shown in U.S. Pat. No. 7,171,935 to Komai, have been treated so that the exterior surface of the liner has a series of spines extending out from the liner. Other liners, such as U.S. Pat. No. 7,665,440 to Holtan et al. describe grit-blasting the outer surface of the cylinder liner so that the outer surface has cavities throughout. German Patent No. DE102009043566A1 to Bischofberger et al. describes a cylinder liner that is created with a textured surface that can have grooves, ribs, shafts, studs, mushrooms, thorns or a combination thereof. This texture can be created by removing material from the liner or by a coating.

U.S. Pat. No. 8,402,881 to Sato et al. discloses an insert casting structure having a rough-cast surface with spines of specific diameters. Based on the measurements, it can be determined that the spines have a more or less cylindrical shape.

## SUMMARY OF THE INVENTION

The present invention relates to a cylinder liner for internal combustion engines that has an outer roughened surface that has particularly good adherence properties. The surface is covered with protrusions or spines of varying shapes and sizes, which are created by spraying the mold with a coating and then casting the cylinder liner in the mold. The spines are generally conical or needle-shaped, with the bases being larger than the tips.

The coating can be formed by spraying the mold used to cast the cylinder liner with a coating material during a centrifugal casting process. First, the mold is sprayed with the coating while rotating so that the mold surface is coated evenly. Then, the casting material is poured into the mold and allowed to solidify. The mold is rotating during the coating, casting and solidifying process.

The coating is prepared in such a way that spines of a specific shape, size and pattern are arranged around the cylinder. These spines are preferably arranged in a density of

## 2

between 110-190 spines/cm<sup>2</sup> and preferably around 120-125 spines/cm<sup>2</sup>. The spines preferably have a surface area of the rough structure compared to the cylindrical ground surface of 120-180%. Due to the conical nature of the spines, it is possible also to measure the surface area covered by the spines at certain heights as compared to the overall cylindrical ground surface. In the present invention, the surface area covered by the spines at 0.2 mm height is approximately 50-90% of the cylindrical ground surface. This area at 0.4 mm height is between 20-45% of the area of the cylindrical ground surface. The distance between the spines as measured from their peaks ranges between 0.09-1.52 mm, with an average distance of 0.64 mm.

## BRIEF DESCRIPTION OF THE DRAWINGS

Other objects and features of the present invention will become apparent from the following detailed description considered in connection with the accompanying drawings. It is to be understood, however, that the drawings are designed as an illustration only and not as a definition of the limits of the invention.

In the drawings, wherein similar reference characters denote similar elements throughout the several views:

FIG. 1 shows a view of cylinder liner according to the invention;

FIG. 2 is a section of a cylinder according to the present invention;

FIG. 3 is a topographical cross-section at 0.2 mm from the cylindrical ground surface of the cylinder of FIG. 2;

FIG. 4 is a topographical cross section at 0.44 mm from the cylindrical ground surface of the cylinder of FIG. 2;

FIG. 5 shows radial cross sections of the cylinder of FIG. 2, taken 1 mm apart.

FIG. 6 is a section of another cylinder according to the present invention;

FIG. 7 is a topographical cross-section at 0.2 mm from the cylindrical ground surface of the cylinder of FIG. 6;

FIG. 8 is a topographical cross section at 0.44 mm from the cylindrical ground surface of the cylinder of FIG. 6;

FIG. 9 shows radial cross sections of the cylinder of FIG. 6, taken 1 mm apart;

FIG. 10 is a section of a cylinder according to the present invention;

FIG. 11 is a topographical cross-section at 0.2 mm from the cylindrical ground surface of the cylinder of FIG. 10;

FIG. 12 is a topographical cross section at 0.44 mm from the cylindrical ground surface of the cylinder of FIG. 10;

FIG. 13 shows radial cross sections of the cylinder of FIG. 10, taken 1 mm apart;

FIG. 14 is a section of a cylinder according to the present invention;

FIG. 15 is a topographical cross-section at 0.2 mm from the cylindrical ground surface of the cylinder of FIG. 14;

FIG. 16 is a topographical cross section at 0.44 mm from the cylindrical ground surface of the cylinder of FIG. 14;

FIG. 17 shows radial cross sections of the cylinder of FIG. 14, taken 1 mm apart;

FIG. 18 is a section of a cylinder according to the present invention;

FIG. 19 is a topographical cross-section at 0.2 mm from the cylindrical ground surface of the cylinder of FIG. 18;

FIG. 20 is a topographical cross section at 0.44 mm from the cylindrical ground surface of the cylinder of FIG. 18;

FIG. 21 shows radial cross sections of the cylinder of FIG. 18, taken 1 mm apart;

FIG. 22 is a topographical section of another cylinder liner, shown at the peaks of the spines;

FIG. 23 is a topographical section of another cylinder liner, shown at the peaks of the spines.

#### DETAILED DESCRIPTION OF THE PREFERRED EMBODIMENTS

As shown in FIG. 1, cylinder liner 1 according to the invention has a roughened surface 2 formed from spines of generally conical or needle shape, with a surface area of the base of the spines being larger than a surface area at a midpoint or tip of the spines.

To form cylinder liner 1, a coating is applied to the mold used to cast the cylinder liner, so that the coating imprints its structure onto the cast cylinder liner. A centrifugal casting method is used to cast the liner so that the exterior of the liner is imprinted with spines of specific size, shape and density. The spines generally have a height of between 0.1-1.1 mm and a density of between 110-300 spines/cm<sup>2</sup>. In one form, the spines have a height of between 0.25-0.85 mm and a density of between 110-190 spines/cm<sup>2</sup>. The density may be adjusted through various processing steps of the coating and how it is applied to the mold. The density of the spines may be adjusted to accommodate the processing and mold technique of the engine block to ensure proper seating and interconnection between the liner and the engine block. For example, if the engine block is molded using high pressure die casting technique the liner may have a higher density of spines and in one example is in the range of 160-200 spines/cm<sup>2</sup>.

Other engine block molding techniques such as precision gravity sand cast or low pressure sand cast the liner spine geometry may include a lower density of spines allowing for an increase opening or spacing between the spines to facilitate the flow of the engine block material into the spines structures before the setting of the material around the cylinder liners. In the lower pressure sand casting techniques the liner may have a spine density of 120-160 spines/cm<sup>2</sup>.

FIGS. 2-21 show sections of the cast cylinder liner according to the invention, as well as topographic images of sections of the liner at 0.2 mm and 0.4 mm from the base and cross-sectional views of the spines. For example, FIG. 2 shows a section of roughened surface 2 having a surface area

covered. As can be seen in FIG. 4, the cylindrical cross-section is taken at 0.4 mm from the cylinder ground diameter shows only 23.1% coverage. Radial cross-sections of the spines at 1 mm intervals across the cylinder can be seen in FIG. 5. The unique worm-like or volcano-shaped spines of the present invention also have an increased perimeter measurement in comparison to a circular or oval shaped spine.

FIGS. 6-9 show another section of a roughened surface 2 of a cylinder liner according to the invention. This section has a cross-sectional surface area at 0.2 mm that covers 77.6% of the cylindrical ground surface (FIG. 7) and a cross-sectional surface area at 0.4 mm that covers 29.8% of the cylindrical ground surface (FIG. 8). The spine configuration at radial cross sections can be seen in FIG. 9.

FIGS. 10-13 show another roughened surface 2 of a cylinder liner section according to the invention, this one having a cross-sectional surface area at 0.2 mm (FIG. 11) that covers 76.2% of the cylindrical ground surface and a cross-sectional surface area at 0.4 mm (FIG. 12) that covers 21.0% of the cylindrical ground surface. The spine configuration at radial cross sections can be seen in FIG. 13.

FIGS. 14-17 show another cylinder liner section, this one having a cross-sectional surface area at 0.2 mm (FIG. 15) that covers 67.8% of the cylindrical ground surface and a cross-sectional surface area at 0.4 mm (FIG. 16) that covers 26.4% of the cylindrical ground surface. The spine configuration at radial cross sections can be seen in FIG. 17.

FIGS. 18-21 show another cylinder liner section, this one having a cross-sectional surface area at 0.2 mm (FIG. 19) that covers 83.3% of the cylindrical ground surface and a cross-sectional surface area at 0.4 mm (FIG. 20) that covers 40.2% of the cylindrical ground surface. The spine configuration at radial cross sections can be seen in FIG. 21.

The spines are arranged so that they are separated by a defined distance, preferably 0.09-1.52 mm.

FIGS. 22-23 show topographical images of the spines and distance measurements between peaks of the spines in the cylinder liner according to the invention taken in a 2 mm<sup>2</sup> section. The spine dimensions are also measured at the peak of each spine.

Table 1 shows the dimensions the spines in the section shown in FIG. 22.

TABLE 1

|           | Short Dimension (mm) | Long Dimension (mm) | Area (mm <sup>2</sup> ) | Perimeter (mm) | Circularity $\frac{4\pi \times \text{Area}}{(\text{Perimeter})^2}$ | Spine Distance (mm) |
|-----------|----------------------|---------------------|-------------------------|----------------|--------------------------------------------------------------------|---------------------|
| Average   | 0.22                 | 0.31                | 0.05                    | 1.12           | 0.50                                                               | 0.76                |
| Median    | 0.22                 | 0.29                | 0.05                    | 1.08           | 0.51                                                               | 0.71                |
| Std. Dev. | 0.06                 | 0.09                | 0.03                    | 0.33           | 0.10                                                               | 0.41                |
| Max       | 0.43                 | 0.54                | 0.15                    | 2.08           | 0.71                                                               | 1.52                |
| Min       | 0.12                 | 0.13                | 0.01                    | 0.45           | 0.26                                                               | 0.11                |

rough structure compared to the cylindrical ground diameter surface of 125%. As shown in FIG. 3, the cylindrical cross section is taken at a 0.2 mm radial distance from the ground diameter shows that 73.2% of the surface is covered with spines. The spines have a needle-like or cone-like structure, so at higher points along the spine, less of the cylinder is

The spines in the liner shown in FIG. 22 are separated by a distance of between 0.11-1.52 mm.

Table 2 shows the spine dimensions and density of another cylinder liner according to the invention, taken in a section shown in FIG. 23.

TABLE 2

|           | Short Dimension (mm) | Long Dimension (mm) | Area (mm <sup>2</sup> ) | Perimeter (mm) | Circularity $\frac{4\pi \times \text{Area}}{(\text{Perimeter})^2}$ | Spine Distance (mm) |
|-----------|----------------------|---------------------|-------------------------|----------------|--------------------------------------------------------------------|---------------------|
| Average   | 0.22                 | 0.30                | 0.05                    | 1.11           | 0.49                                                               | 0.55                |
| Median    | 0.21                 | 0.28                | 0.04                    | 0.99           | 0.49                                                               | 0.49                |
| Std. Dev. | 0.08                 | 0.11                | 0.04                    | 0.43           | 0.06                                                               | 0.29                |
| Max       | 0.48                 | 0.67                | 0.21                    | 2.71           | 0.64                                                               | 1.33                |
| Min       | 0.12                 | 0.15                | 0.01                    | 0.53           | 0.34                                                               | 0.09                |

Here, the spines are separated by a distance of between 0.09-1.33 mm.

Table 3 shows the spine dimensions and density of another cylinder liner according to the invention, taken in a section. Here, the spines have a distance of between 0.18-1.3 mm.

What is claimed is:

1. A cast cylinder liner for an internal combustion engine, having an outer surface with a plurality of spines disposed thereon in an irregular pattern, the spines having an aggregate cross-sectional surface area measured at 0.2 mm from a ground cylindrical surface that is between 50-90% of the

TABLE 3

|           | Short Dimension (mm) | Long Dimension (mm) | Area (mm <sup>2</sup> ) | Perimeter (mm) | Circularity $\frac{4\pi \times \text{Area}}{(\text{Perimeter})^2}$ | Spine Distance (mm) |
|-----------|----------------------|---------------------|-------------------------|----------------|--------------------------------------------------------------------|---------------------|
| Average   | 0.21                 | 0.28                | 0.04                    | 1.00           | 0.55                                                               | 0.63                |
| Median    | 0.21                 | 0.27                | 0.04                    | 0.94           | 0.55                                                               | 0.57                |
| Std. Dev. | 0.04                 | 0.07                | 0.02                    | 0.22           | 0.07                                                               | 0.30                |
| Max       | 0.30                 | 0.47                | 0.08                    | 1.44           | 0.69                                                               | 1.30                |
| Min       | 0.13                 | 0.17                | 0.02                    | 0.57           | 0.40                                                               | 0.18                |

30

Table 4 shows aggregate data for all three sections described above. The spines according to the invention have a separation of between 0.09-1.52 mm, with a median distance of 0.59 mm, measured from the peak of one spine to the peak of an adjacent spine.

total ground cylindrical surface area, and an aggregate cross-sectional surface area measured at 0.4 mm from the ground cylindrical surface that is between 20-45% of the total ground cylindrical surface area, wherein the spines vary in cross-section and distances from one another, wherein a

TABLE 4

|           | Short Dimension (mm) | Long Dimension (mm) | Area (mm <sup>2</sup> ) | Perimeter (mm) | Circularity $\frac{4\pi \times \text{Area}}{(\text{Perimeter})^2}$ | Spine Distance (mm) |
|-----------|----------------------|---------------------|-------------------------|----------------|--------------------------------------------------------------------|---------------------|
| Average   | 0.22                 | 0.30                | 0.05                    | 1.08           | 0.51                                                               | 0.64                |
| Median    | 0.21                 | 0.28                | 0.04                    | 1.01           | 0.51                                                               | 0.59                |
| Std. Dev. | 0.06                 | 0.09                | 0.03                    | 0.35           | 0.08                                                               | 0.34                |
| Max       | 0.48                 | 0.67                | 0.21                    | 2.71           | 0.71                                                               | 1.52                |
| Min       | 0.12                 | 0.13                | 0.01                    | 0.45           | 0.26                                                               | 0.09                |

The measurements of Tables 1-4 further define the spine geometry and the measurements are summarized for reference. The area refers to the spine area as measured at the tip of each spine. Analysis software is used to determine the various geometries of the spines. One of these determinations is a basis to classify the circularity of the spine. The software may determine the circularity based on a base chart or may be determined on various measurements such as the short and long dimensions of each spine. The software also can quickly determine the spine distance between the spines. The lower spine count and elongated shape of the spines allows for a more open structure and increases the distance between the spines. The increased distance may allow for the casting material of the engine block around the liner to contact the exterior surface and minimize any gaps to improve the heat transfer between the liner into the engine block.

50 distance between at least two of the spines is 0.9 mm and a distance between at least two other of the spines is 1.52 mm and distances between any of the spines and a nearest spine is between 0.9 mm and 1.52 mm.

2. The cast cylinder liner according to claim 1, wherein the distance between the spines averages about 0.64 mm.

55 3. The cast cylinder liner according to claim 1, wherein the cross-sectional surface area of the spines measured at 0.2 mm from the ground cylindrical surface is between 60-85% of the total ground cylindrical surface area, and the cross-sectional surface area of the spines measured at 0.4 mm from the ground cylindrical surface is between 25-40% of the total ground cylindrical surface area.

4. The cast cylinder liner according to claim 1, wherein the cylinder liner has a spine density of 110-300 spines/cm<sup>2</sup>.

5. The cast cylinder liner according to claim 4, wherein the cylinder liner has a spine density of 120-160 spines/cm<sup>2</sup>.

60 6. The cast cylinder liner according to claim 4 wherein the cylinder liner has a spine density of 160-200 spines/cm<sup>2</sup>.

7. The cast cylinder liner according to claim 1, wherein the cylinder liner has a surface area of a rough structure covered with spines of 120-180% of the cylindrical ground surface area.

8. The cast cylinder liner according to claim 1, wherein the cylinder liner has a spine height of 0.1 mm to 1.1 mm.

9. The cast cylinder liner according to claim 1, wherein the cylinder has a spine height of 0.3-0.7 mm.

10. A cast cylinder liner for an internal combustion engine, having an outer surface with a plurality of conically shaped spines disposed thereon in an irregular pattern, the spines having an aggregate cross-sectional surface area measured at 0.2 mm from a ground cylindrical surface that is between 50-90% of the total ground cylindrical surface area, and an aggregate cross-sectional surface area measured at 0.4 mm from the ground cylindrical surface that is between 20-45% of the total ground cylindrical surface area, wherein the spines vary in cross-section and distances from one another, wherein distances between adjacent spines measured at their peak are between 0.09-1.52 mm and wherein the distance between the adjacent spines averages about 0.64 mm.

\* \* \* \* \*